# EUROPEAN PATENT SPECIFICATION

(11) **EP 4 156 214 B1**
(45) Date of publication and mention of the grant of the patent: **21.05.2025**
(21) Application number: 22194858.1
(22) Date of filing: 09.09.2022
(51) Int. Cl.: H01F 41/02, H01F 1/057

(54) **MANUFACTURING METHOD OF A LOW-HEAVY RARE EARTH MAGNET**
HERSTELLUNGSVERFAHREN EINES SELTENERDMAGNETEN MIT GERINGEN SCHWEREN SELTENERDEN
PROCÉDÉ DE FABRICATION D'UN AIMANT DE TERRES RARES À FAIBLE TENEUR EN TERRES RARES LOURDES

(30) Priority: 24.09.2021 CN 202111121038
(43) Date of publication of application: 29.03.2023
(73) Proprietor: Yantai Dongxing Magnetic Materials Inc., Yantai City 265500 (CN)
(72) Inventor: Wang, Chuanshen, Yantai City 265500 (CN); Peng, Zhongjie, Yantai City 265500 (CN); Yang, Kunkun, Yantai City 265500 (CN); Ding, Kaihong, Yantai City 265500 (CN)
(74) Representative: Gulde & Partner

(56) References cited:
- WO-A1-2013/072728
- CN-A- 111 916 284
- CN-A- 112 863 848
- US-A1- 2013 195 710
- US-A1- 2018 247 743
- US-B2- 10 109 403

## Description

### BACKGROUND OF THE INVENTION

### 1. Field of the Invention

The invention relates to the technical field of sintered type NdFeB permanent magnets, in particular to a low-cost rare earth magnet and a corresponding manufacturing method thereof.

### 2. Description of the Prior Art

NdFeB sintered permanent magnets are widely used in high-tech fields such as electronic equipment, medical equipment, electric vehicles, household products, robots, etc. In the past few decades of development, NdFeB permanent magnets have been rapidly developed and the residual magnetic properties have basically reached the theoretical limit. However, the gap between the coercive force and the theoretical value is still very large, so improving the coercive force of the magnet is a major research hotspot.

Heavy rare earths terbium (Tb) or Dysprosium (Dy) are added for greatly improving the magnetic coercivity of the NdFeB magnets. According to one conventional manufacturing process, Tb or Dy are directly mixed into the magnet alloy powders, but consume large amounts of Tb or Dy thereby significantly increasing the material costs. According to an improved manufacturing process, the amount of Tb or Dy can be greatly reduced by applying the grain boundary diffusion technology, but still the material costs are very high for the heavy rare earths. Therefore, it is still important to continuously reduce the total content of heavy rare earths in the NdFeB magnet.

Although increasing the coercivity is most effective through diffusing heavy rare earths, the abundance of heavy rare earths is low and accordingly the price is expensive. Therefore, more and more researchers are preparing heavy rare earth alloys with low melting point to obtain with improved coercivity.

CN106024253A discloses NdFeB magnets which are diffused with Tb, Dy or Ho, contain an M2 boride phase, an HR enrichment layer and a specific core-shell structure including an (R,HR)-Fe(Co)-M1 phase covering the main phase. In CN108305772A the diffusion source is a hydride powder of an R1 - R2-M type alloy, whose melting point is 400-800 °C. CN111524674A provides a magnet characterized by a grain-bounded epitaxial layer, namely a two-particle boundary phase R_{X}Ho_{y}Cu_{Z}X1, is proposed to greatly increase the performance of the magnet after diffusion.

Further examples may be found in US 2018/247743 A1, US 2013/195710 A1, US 10 109 403 B2, CN 111 916 284 A, CN 112 863 848 A and WO 2013/072728 A1. US 2018/247743 A1 and US 2013/195710 A1 disclose that mixing the pulverized magnetic powder with a non-magnetic low melting point (LMP) alloy powder are consolidated or sintered into a bulk magnet. Firstly, the method is easy to result in inhomogeneous distribution of the NdFeB. Secondly, The RM alloy is well known skilled person. The ratio of RM alloy to the NdFeB is the difficult point and the method applied also is critical. The traditional method of mixing the pulverized magnetic powder with RM alloy powder can not get low melting point grain boundaries uniformly. And the diffusion source is diffused into the magnet unevenly and results in poor performance of NdFeB. Designing magnets with low melting point grain boundaries and coordinating with multiple diffusion sources is important.

In the above techniques, the magnets are to form a specific phase or use low-cost diffusion sources for reducing the production cost of the magnets. However, there is still a need to further reduce the content of heavy rare earths of NdFeB magnets.

### SUMMARY OF THE INVENTION

The invention is defined by the appended claims. The description that follows is subjected to this limitation. Any disclosure lying outside the scope of said claims is only intended for illustrative as well as comparative purposes.

There is provided a method of preparing a sintered NdFeB magnet as defined in claim 1.

Further embodiments of the invention could be learned form the dependent claims and the following description.

### BRIEF DESCRIPTION OF THE FIGURES

Figure 1 shows a SEM image using ZISS electron microscopy of the microstructure of an exemplary Nd-Fe-B permanent magnet after diffusion and aging.

### DETAILED DESCRIPTION OF THE INVENTION

Reference will now be made in detail to embodiments. The present disclosure, however, may be embodied in various different forms, and should not be construed as being limited to only the illustrated embodiments herein. Rather, these embodiments are provided as examples so that this disclosure will be thorough and complete, and will fully convey the aspects and features of the present disclosure to those skilled in the art.

### General Procedure

The present invention provides a low-heavy rare earth magnet (i.e. a sintered NdFeB magnet including a low content of heavy rare earth elements) and a corresponding manufacturing method. A special diffusion source for the diffusion process is coated onto a sintered NdFeB magnet of a well-defined magnet composition. Diffusion and aging results to the formation of a high-performance magnet with a specific phase structure. Even in the presence of reduced heavy rare earth contents, the magnet shows a greatly increased coercivity. It is assumed that the combination of the specific grain boundary structure and the diffusion source can greatly improve the coercivity.

There is provided a method of preparing a sintered NdFeB magnet comprising the following steps:
(S1) Smelting of the raw materials of a NdFeB alloy to obtain strip casting NdFeB alloy sheets and mechanically crushing the NdFeB alloy sheets into flake alloy sheets, wherein the NdFeB alloy has the following composition in weight percentage:
   28%≤R≤30%, 0.8%≤B≤1.2%, 0≤Gd≤5%, 0≤Ho≤5%, and 0≤M≤3%,
   where R is at least one element of Nd, Pr, Ce, La, Tb, and Dy,
   M is at least one element of Co, Mg, Ti, Zr, Nb, and Mo, and
   the rest of the NdFeB alloy is Fe;
(S2) Mechanically mixing the flake alloy sheets, a low melting point powder and a lubricant, followed by hydrogen absorption and dehydrogenation treatment of the mixture and jet milling of the product to obtain a NdFeB magnet powder, wherein the low melting point powder contains at least one component selected form NdCu, NdAl and NdGa and a weight percentage of the components is 0%≤NdCu≤3%, 0%≤NdAl≤3%, and 0%≤NdGa≤3% with respect to the total weight of the flake alloy sheets and the low melting point powder;
(S3) Pressing and forming the NdFeB powder to a blank and sintering the blank to obtain a sintered NdFeB magnet;
(S4) Mechanically processing the sintered NdFeB magnet to a desired shape, and then forming a diffusion source film on the surface of the sintered NdFeB magnet, wherein diffusion source film includes a diffusion source of formula RₓH_{y}M_{1-x-y}, wherein
   R is at least one of Nd, Pr, Ce, La, Ho, and Gd,
   H is at least one of Tb and Dy,
   M is at least one of Al, Cu, Ga, Ti, Co, Mg, Zn, and Sn, and
   where x and y are set to be 10%<x≤50% and 40%<y≤70% in weight percentage; and
(S5) Performing a diffusion process and aging to obtain the final the sintered NdFeB magnet.

According to one embodiment, in step (S2) a weight content of Cu is 0.1%≤Cu≤0.5%, a weight content of Al is 0.2%≤Al≤0.9%, and a weight content of Ga is 0.01%≤Ga≤0.4%, each with respect to the total weight of the flake alloy sheets and the low melting point powder.

According to another embodiment, in the NdFeB alloy of step (S1) R is at least one element of Nd and Pr, and M is at least one element of Co and Ti. Further, the NdFeB alloy sheets may be mechanically crushed into flake alloy sheets of 150 - 400µm.

According to another embodiment, in the diffusion source of step (S4)
R is at least one of Nd and Pr,
H is Dy, and
M is at least one of Al, Cu, and Ga.

In step (S2), the dehydrogenation temperature is 400 - 600 °C.

According to another embodiment, in step (S2), an average particle size D50 of the low melting point powder is 200 nm - 4 µm measured by laser diffraction (LD). Further, an average particle size D50 of the NdFeB magnet powder may be 3 - 5 µm after jet milling measured by laser diffraction (LD). The measurement method may be performed according to ISO 13320-1. According to the IUPAC definition, the equivalent diameter of a non-spherical particle is equal to a diameter of a spherical particle that exhibits identical properties to that of the investigated non-spherical particle.

According to another embodiment, in step (S3), the sintering temperature of the NdFeB magnet is 980 - 1060 °C and the sintering time is 6 - 15h.

According to another embodiment, in step (S5), the diffusion temperature of NdFeB magnets is 850 - 930 °C and the diffusion time is 6 - 30h.

According to another embodiment, in step (S5), an aging temperature is 420 - 680 °C, an aging time is 3 - 10h, an aging heating rate is 1 - 5 °C/min, and an aging cooling rate is 5 - 20 °C/min.

A sintered NdFeB magnet is obtained by the above-mentioned preparation method.

A phase structure of the sintered NdFeB magnet may comprise:
a main phase;
an R shell consisting of at least one of Nd, Pr, Ce, La, Ho, and Gd and partially covering the main phase;
a transition metal shell consisting of at least one of Cu, Al, and Ga and partially covering the main phase; and
a triangular region consisting of at least one composition of Formulae 1 - 3:

   Formula 1 NdₐFe_{b}R_{c}M_{d},

   wherein R is at least one element of Pr, Ce, La, Ho, and Gd
   M is at least three elements of Al, Cu, Ga, Ti, Co, Mg, Zn, and Sn, and
   where a, b, c, and d are set to be 30%≤a≤70%, 5%≤b≤40%, 5%≤c≤35%, and 0%≤d≤15% in weight percentage;

      Formula 2 NdₑFe_{f}R_{g}HₕKᵢMⱼ

      wherein R is at least one element of Pr, Ce, La,
      H is at least one element of Dy and Tb,
      M is at least three elements of Al, Cu, Ga, Ti, Co, Mg, Zn, and Sn, and
      where e, f, g, h, I, and j are set to be 25%≤e≤65%, 5%≤f≤35%, 5%≤g≤30%, 5%≤h≤30%, 5%≤i≤10%, and 0%≤j≤10% in weight percentage;

         Formula 3 NdₖFeₗRₘDₙMₒ

         wherein R is at least one element of Pr, Ce, La, Ho, and Gd,
         D is at least one element of Al, Cu, and Ga,
         M is at least one element of Ti, Co, Mg, Zn, and Sn, and
         where k, l, m, n, and o are set to be 30%≤k≤70%, 5%≤l≤35%, 5%≤m≤35%, 5%≤n≤25%,
         and 0%≤o≤10% in weight percentage. The diffusion source may be uniformly distributed in the RH phase and RHM phase.

A thickness of the obtained sintered NdFeB magnet may be 0.3 - 6 mm.

(S2) The flake alloy sheets, low melting point powders and lubricant for mechanical mixing and stirring are put into the hydrogen treatment furnace for hydrogen absorption and dehydrogenation treatment. The NdFeB magnet powders are prepared by jet milling.

(S3) The NdFeB magnet are prepared by magnetic field orientation molding, sintering treatment.

(S4) The NdFeB magnet is machined into the desired shape after sintering, and then a low-heavy rare earth diffusion source film are coated with the NdFeB magnet.

(S5) The Low-heavy rare earth magnets are prepared by diffusion and aging processing.

Preferably, wherein: in step (S1), the NdFeB alloy raw material compositions of weight percentage are, respectively, 28% ≤ R≤30%, 0.8% ≤ B≤ 1.2%, 0≤Gd≤5%,0≤Ho≤5%,0% ≤M≤3%, the R including at least two elements of Nd, Pr, Ce, La, Tb, Dy, the M including at least one element of Co, Mg, Ti, Zr, Nb, Mo, the rest is Fe. The mixed low melting point powders contain NdCu, NdAl and NdGa, whose weight percentage is 0%≤NdCu≤3%, 0%≤NdAl≤3%, 0%≤NdGa≤3%.

Preferably, a low-heavy rare earth diffusion source is atomized milling, amorphous alloy sheets or ingot casting.

Preferably, wherein: in step (S2), the dehydrogenation temperature is 400 - 600 °C.

Preferably, wherein: in step (S2), the particle size of the low melting point powders is 200 nm - 4 µm. The particle size of NdFeB magnets alloy powders is 3 - 5 µm after jet milling.

Preferably, wherein: in step (S3), the sintering temperature of NdFeB magnets is 980 - 1060 °C, the sintering time is 6 - 15h;
Preferably, wherein: in step (S5), the diffusion temperature of NdFeB magnets is 850 - 930 °C, the diffusion time is 6 - 30h, the aging temperature is 420 - 680 °C, and the aging time is 3 - 10h. The aging temperature of the NdFeB magnet is heated at a rate of 1 - 5°C/min, and the cooling rate is 5 - 20 °C/min.

The beneficial effects of using the above further scheme are:
A grain boundary magnet with low melting point is designed and a special diffusion source with special phase structure are coated with the magnet. A low-heavy rare earth NdFeB magnet with specific grain boundary structure is obtained by diffusion and aging treatment; The coercivity is greatly improved through the synergy of magnet composition and diffusion source.

The diffusion magnet matrix contains NdCu, NdAl and NdGa of the low melting point phase, which is conducive to increasing the diffusion coefficient of the magnet grain boundary, thereby improving the diffusion efficiency of the diffusion source;
The crystal phase structure distribution of the diffusion source is the RM phase and RHM phase, which can improve the diffusion coefficient, therefore it is beneficial to enter the magnet for the element of the diffusion source. This way can well form a magnetic isolation effect in the low-heavy rare earth NdFeB magnet, and realize the role of improving the coercivity.

The low-heavy rare earth magnet has a characteristic phase, and the characteristic phase Fe mass content <30%, which has non-ferromagnetic properties and can have a good magnetic isolation effect;
The present invention can reduce the heavy rare earth content in the magnet very well, can greatly reduce the cost of the magnet, the process is simple, can achieve mass production.

### Exemplary Embodiments

The preparation process of exemplary sintered NdFeB magnets will now be described in detail.

NdFeB alloy raw materials are mixed with different ratios of NdCu, NdAl, and NdGa and a conventional lubricant is added. Magnet compositions No. 1 - 22 are summarized in Table 1 below.

The preparation method of the NdFeB alloy was as follows:
The NdFeB alloy raw materials are smelted in a strip casting process to obtain NdFeB alloy sheets, and the obtained alloy sheets are mechanically crushed into flake alloy sheets of 150 - 400µm size.

NdCu, NdAl and NdGa as low melting point powders with a particle size range of 200 nm - 4 µm are mixed and added to the flake alloy sheets.

The mixed materials of the flake alloy sheets, low melting point powders and lubricant are put into the hydrogen treatment furnace for hydrogen absorption and dehydrogenation treatment, wherein the dehydrogenation temperature is 400 - 600 °C. The low melting point alloy powders are coating the flake alloy sheets. NdFeB powders are prepared by air milling and the NdFeB powder particle size is 3 - 5 µm.

The addition of a lubricant during the jet milling step is well-known. Any common type of lubricant und its dosage can be used. There is no specific restriction.

The NdFeB alloy powders after the air flow grinding is oriented molding and pressed into the blank by isostatic pressure.

The pressing blank of NdFeB is sintered in vacuum, and quickly cooled by argon, and then the blank is heat-treated including a primary tempering and secondary aging. The sintered magnet performance is tested, and the specific process conditions and magnet characteristic are shown in Table 2.

The sintered NdFeB magnet is mechanically processed to obtain the desired shape and then a diffusion source film is coated on the sintered NdFeB magnet. The weight of Dy on the sintered NdFeB magnet is 1.0wt.%, and the weight of Dy in Dy alloy on the sintered NdFeB magnet is 1.0wt.%.

An increase in coercivity after diffusion of the Dy alloy reaches 636.8 - 756.2 kA/m, and the process allows to reduce the production cost of the magnet due to the low Dy content.

The diffusion sources based on Dy alloys and magnet characteristics of the sintered NdFeB magnets are shown in Table 3.

Pure diffusion examples of Dy and magnet characteristics of the sintered NdFeB magnets are shown in Table 4.

**Table 1 - Magnet compositions resulting from the combination of NdFeB alloy flakes and low melting point powders**

| | Magnet composition | | | | | | | | | | |
|---|---|---|---|---|---|---|---|---|---|---|---|
| Number | Al | B | Co | Cu | Fe | Ga | Nd | Pr | Ti | Ho | TRE |
| 1 | 0.30% | 0.97% | 1.00% | 0.15% | Margin | 0.05% | 29.52% | | | | 29.52% |
| 2 | 0.59% | 0.95% | 1.00% | 0.15% | Margin | 0.11% | 31.23% | | | | 31.23% |
| 3 | 0.87% | 0.93% | 1.00% | 0.14% | Margin | 0.21% | 33.19% | | | | 33.19% |
| 4 | 0.83% | 0.95% | 1.00% | 0.29% | Margin | 0.05% | 31.51% | | | | 31.51% |
| 5 | 0.41% | 0.92% | 1.00% | 0.29% | Margin | 0.10% | 26.35% | 6.59% | 0.05% | | 32.94% |
| 6 | 0.53% | 0.95% | 1.00% | 0.29% | Margin | 0.21% | 24.81% | 6.20% | 0.05% | | 31.02% |
| 7 | 0.82% | 0.94% | 1.00% | 0.44% | Margin | 0.05% | 25.61% | 6.40% | 0.05% | | 32.02% |
| 8 | 0.53% | 0.95% | 1.00% | 0.44% | Margin | 0.11% | 24.74% | 6.19% | 0.06% | | 30.93% |
| 9 | 0.35% | 0.92% | 1.00% | 0.43% | Margin | 0.21% | 26.19% | 6.55% | 0.05% | | 32.73% |
| 10 | 0.42% | 0.97% | 1.00% | 0.15% | Margin | 0.11% | 23.89% | 5.97% | 0.10% | | 29.86% |
| 11 | 0.59% | 0.94% | 1.00% | 0.15% | Margin | 0.21% | 31.82% | | 0.10% | | 31.82% |
| 12 | 0.86% | 0.92% | 1.00% | 0.14% | Margin | 0.31% | 33.76% | | 0.10% | | 33.76% |
| 13 | 0.82% | 0.94% | 1.00% | 0.29% | Margin | 0.11% | 23.86% | 7.95% | 0.10% | | 31.81% |
| 14 | 0.41% | 0.91% | 1.00% | 0.29% | Margin | 0.21% | 25.14% | 8.38% | 0.10% | | 33.52% |
| 15 | 0.53% | 0.94% | 1.00% | 0.29% | Margin | 0.32% | 23.71% | 7.90% | 0.20% | | 31.61% |
| 16 | 0.81% | 0.94% | 1.00% | 0.43% | Margin | 0.11% | 32.31% | | 0.20% | | 32.31% |
| 17 | 0.53% | 0.94% | 1.00% | 0.44% | Margin | 0.21% | 31.52% | | 0.20% | | 31.52% |
| 18 | 0.35% | 0.91% | 1.00% | 0.43% | Margin | 0.31% | 33.31% | | 0.20% | | 33.31% |
| 19 | 0.31% | 0.97% | 0.91% | 0.20% | Margin | 0.18% | 24.83% | 6.39% | 0.20% | | 31.22% |
| 20 | 0.70% | 1.00% | 1.00% | 0.15% | Margin | 0.20% | 25.00% | 6.20% | 0.10% | | 31.20% |
| 21 | 0.34% | 0.91% | 1.00% | 0.15% | Margin | 0.20% | 22.00% | 5.50% | 0.15% | 3.37% | 30.87% |
| 22 | 0.28% | 0.87% | 0.80% | 0.38% | Margin | 0.37% | 23.62% | 7.60% | 0.10% | | 31.22% |

**Table 2 - Process conditions and sintered NdFeB magnet performance**

| Number | Sintering temp. | holding time | One-level aging | holding time | Secondary aging | holding time | Heating rate | Cooling rate | Performance | | |
|---|---|---|---|---|---|---|---|---|---|---|---|
| | °C | h | °C | h | °C | h | °C/min | °C/min | Br(T) | Hcj (kA/m) | Hk/Hcj |
| 1 | 980 | 15 | 850 | 3 | 450 | 3 | 5 | 5 | 14.55 | 14.29 | 0.99 |
| 2 | 980 | 15 | 850 | 3 | 450 | 3 | 5 | 5 | 13.86 | 16.72 | 0.99 |
| 3 | 980 | 15 | 850 | 3 | 450 | 3 | 5 | 10 | 13.17 | 19.42 | 0.97 |
| 4 | 980 | 15 | 850 | 3 | 450 | 3 | 5 | 15 | 13.56 | 17.48 | 0.98 |
| 5 | 980 | 15 | 850 | 3 | 480 | 3 | 3 | 15 | 13.67 | 16.49 | 0.98 |
| 6 | 1020 | 13 | 850 | 3 | 480 | 3 | 1 | 5 | 13.93 | 16.69 | 0.98 |
| 7 | 1020 | 13 | 850 | 3 | 480 | 3 | 1 | 20 | 13.47 | 17.68 | 0.97 |
| 8 | 1020 | 13 | 850 | 3 | 480 | 3 | 3 | 20 | 13.96 | 16.15 | 0.97 |
| 9 | 1020 | 13 | 850 | 3 | 510 | 3 | 3 | 20 | 13.74 | 16.65 | 0.98 |
| 10 | 1020 | 13 | 850 | 3 | 510 | 3 | 3 | 10 | 14.32 | 15.12 | 0.98 |
| 11 | 1040 | 9 | 850 | 3 | 510 | 3 | 1 | 10 | 13.71 | 17.26 | 0.97 |
| 12 | 1040 | 9 | 850 | 3 | 510 | 3 | 1 | 10 | 13.02 | 19.90 | 0.98 |
| 13 | 1040 | 9 | 850 | 3 | 550 | 3 | 5 | 10 | 13.45 | 18.90 | 0.98 |
| 14 | 1040 | 9 | 850 | 3 | 550 | 3 | 5 | 15 | 13.52 | 17.25 | 0.98 |
| 15 | 1040 | 9 | 850 | 3 | 550 | 3 | 5 | 15 | 13.77 | 17.52 | 0.98 |
| 16 | 1060 | 6 | 850 | 3 | 550 | 3 | 3 | 20 | 13.38 | 18.06 | 0.97 |
| 17 | 1060 | 6 | 850 | 3 | 580 | 3 | 1 | 20 | 13.80 | 16.93 | 0.97 |
| 18 | 1060 | 6 | 850 | 3 | 580 | 3 | 3 | 20 | 13.58 | 17.40 | 0.98 |
| 19 | 1060 | 6 | 850 | 3 | 580 | 3 | 3 | 5 | 13.70 | 18.50 | 0.98 |
| 20 | 1060 | 6 | 850 | 3 | 660 | 3 | 1 | 5 | 13.40 | 19.00 | 0.98 |
| 21 | 1050 | 12 | 850 | 3 | 660 | 3 | 1 | 5 | 13.30 | 18.00 | 0.99 |
| 22 | 1060 | 7 | 850 | 3 | 660 | 3 | 1 | 15 | 13.60 | 20.00 | 0.99 |

**Table 3 - Diffusion sources, process conditions and resulting magnet properties**

| Exa mple | Diffusion Source | Size(mm) | Diffusion Temp.°C | holding time hours | Aging Temp. °C | holding time hours | Heating rate °C/min | Cooling rate °C/min | Performance after Diffusion | | |
|---|---|---|---|---|---|---|---|---|---|---|---|
| | | | | | | | | | Br(T) | Hcj (kA/m) | Hk/Hcj |
| 1 | PrDyCu | 10*10*3 | 850 | 30 | 420 | 10 | 5 | 5 | 1.435 | 1950.2 | 0.97 |
| 2 | PrDyCu | 10*10*3 | 850 | 30 | 480 | 7 | 5 | 5 | 1.362 | 2029.8 | 0.97 |
| 3 | PrDyCu | 10*10*3 | 850 | 30 | 500 | 5 | 5 | 10 | 1.295 | 2149.2 | 0.96 |
| 4 | PrDyCu | 10*10*3 | 880 | 20 | 450 | 8 | 5 | 15 | 1.332 | 1990 | 0.96 |
| 5 | NdDyCu | 10*10*4 | 880 | 20 | 500 | 6 | 3 | 15 | 1.342 | 2069.6 | 0.96 |
| 6 | NdDyCu | 10*10*4 | 880 | 20 | 600 | 5 | 1 | 5 | 1.37 | 1990 | 0.97 |
| 7 | NdDyCu | 10*10*4 | 880 | 20 | 500 | 3 | 1 | 20 | 1.325 | 2109.4 | 0.96 |
| 8 | PrDyCu | 10*10*4 | 900 | 15 | 450 | 8 | 3 | 20 | 1.375 | 2029.8 | 0.96 |
| 9 | PrDyCu | 10*10*5 | 900 | 16 | 500 | 6 | 3 | 20 | 1.35 | 2069.6 | 0.97 |
| 10 | PrDyCu | 10*10*5 | 900 | 17 | 520 | 4 | 3 | 10 | 1.41 | 1990 | 0.97 |
| 11 | PrDyCu | 10*10*5 | 900 | 18 | 600 | 5 | 1 | 10 | 1.35 | 1990 | 0.97 |
| 12 | PrDyCu | 10*10*5 | 900 | 19 | 500 | 3 | 1 | 10 | 1.28 | 2189 | 0.97 |
| 13 | PrDyCuGa | 10*10*3 | 910 | 10 | 450 | 8 | 5 | 10 | 1.32 | 2109.4 | 0.96 |
| 14 | PrDyCuGa | 10*10*3 | 910 | 10 | 500 | 6 | 5 | 15 | 1.33 | 2029.8 | 0.97 |
| 15 | PrDyCuGa | 10*10*3 | 910 | 10 | 520 | 4 | 5 | 15 | 1.352 | 2109.4 | 0.97 |
| 16 | PrDyCuAl | 10*10*3 | 910 | 10 | 450 | 5 | 3 | 20 | 1.315 | 2149.2 | 0.97 |
| 17 | PrDyCuAl | 10*10*3 | 910 | 10 | 480 | 3 | 1 | 20 | 1.36 | 1990 | 0.96 |
| 18 | PrDyCuAl | 10*10*3 | 930 | 6 | 450 | 8 | 3 | 20 | 1.332 | 2069.6 | 0.98 |
| 19 | PrDyCu | 10*10*4 | 930 | 6 | 500 | 6 | 3 | 5 | 1.345 | 2149.2 | 0.97 |
| 20 | PrDyCu | 10*10*4 | 930 | 6 | 520 | 4 | 3 | 5 | 1.32 | 2109.4 | 0.97 |
| 21 | PrDyCu | 10*10*4 | 930 | 6 | 600 | 5 | 1 | 5 | 1.305 | 2189 | 0.98 |
| 22 | PrDyCu | 10*10*4 | 930 | 6 | 680 | 3 | 1 | 15 | 1.34 | 2189 | 0.98 |

**Table 4 - Diffusion of Dy, process conditions and properties**

| proportion ality | Diffusion Source | Size (mm) | Diffusion Temp. °C | holding time hours | Aging Temp. °C | holding time hours | Heating rate °C/ min | Coolin g rate ° C/min | Performance after Diffusion | | |
|---|---|---|---|---|---|---|---|---|---|---|---|
| | | | | | | | | | Br(T) | Hcj (kA/m) | Hk/Hcj |
| 1 | Dy | 10*10*3 | 850 | 30 | 420 | 10 | 5 | 5 | 1.436 | 1791.0 | 0.97 |
| 2 | Dy | 10*10*3 | 850 | 30 | 480 | 7 | 5 | 5 | 1.363 | 1870.6 | 0.97 |
| 3 | Dy | 10*10*3 | 850 | 30 | 500 | 5 | 5 | 10 | 1.297 | 1950.2 | 0.96 |
| 4 | Dy | 10*10*3 | 880 | 20 | 450 | 8 | 5 | 15 | 1.333 | 1791.0 | 0.96 |
| 5 | Dy | 10*10*4 | 880 | 20 | 500 | 6 | 3 | 15 | 1.344 | 1910.4 | 0.96 |
| 6 | Dy | 10*10*4 | 880 | 20 | 600 | 5 | 1 | 5 | 1.372 | 1870.6 | 0.97 |
| 7 | Dy | 10*10*4 | 880 | 20 | 500 | 3 | 1 | 20 | 1.326 | 1990.0 | 0.96 |
| 8 | Dy | 10*10*4 | 900 | 15 | 450 | 8 | 3 | 20 | 1.377 | 1910.4 | 0.96 |
| 9 | Dy | 10*10*5 | 900 | 16 | 500 | 6 | 3 | 20 | 1.352 | 1910.4 | 0.97 |
| 10 | Dy | 10*10*5 | 900 | 17 | 520 | 4 | 3 | 10 | 1.411 | 1830.8 | 0.97 |
| 11 | Dy | 10*10*5 | 900 | 18 | 600 | 5 | 1 | 10 | 1.351 | 1751.2 | 0.97 |
| 12 | Dy | 10*10*5 | 900 | 19 | 500 | 3 | 1 | 10 | 1.282 | 1990.0 | 0.97 |
| 13 | Dy | 10*10*3 | 910 | 10 | 450 | 8 | 5 | 10 | 1.322 | 1950.2 | 0.96 |
| 14 | Dy | 10*10*3 | 910 | 10 | 500 | 6 | 5 | 15 | 1.331 | 1910.4 | 0.97 |
| 15 | Dy | 10*10*3 | 910 | 10 | 520 | 4 | 5 | 15 | 1.354 | 1990.0 | 0.97 |
| 16 | Dy | 10*10*3 | 910 | 10 | 450 | 5 | 3 | 20 | 1.316 | 2029.8 | 0.96 |
| 17 | Dy | 10*10*3 | 910 | 10 | 480 | 3 | 1 | 20 | 1.360 | 1870.6 | 0.98 |
| 18 | Dy | 10*10*3 | 930 | 6 | 450 | 8 | 3 | 20 | 1.333 | 1950.2 | 0.97 |
| 19 | Dy | 10*10*4 | 930 | 6 | 500 | 6 | 3 | 5 | 1.346 | 1950.2 | 0.97 |
| 20 | Dy | 10*10*4 | 930 | 6 | 520 | 4 | 3 | 5 | 1.320 | 1990.0 | 0.98 |
| 21 | Dy | 10*10*4 | 930 | 6 | 600 | 5 | 1 | 5 | 1.306 | 1990.0 | 0.98 |
| 22 | Dy | 10*10*4 | 930 | 6 | 680 | 3 | 1 | 15 | 1.340 | 1990.0 | 0.98 |

Based on the above data, the NdCu, NdAl, NdGa phase powders are added to the grain boundary of the NdFeB alloy flakes, whose grain boundary has a low melting point. The grain boundary channel of NdFeB permanent magnets are suitable for the diffusion, especially when the diffusion source is a heavy rare earth alloys. The coercivity increases significantly to △Hcj > 597 kA/m after diffusion, and the coercivity is significantly better than in case of diffusion of pure Dy.

Specifically, the various embodiments of Table 3 and the comparative examples of Table 4 are analyzed as follows:
Example 1, with the same NdFeB magnet composition and size, the same diffusion temperature and aging temperature, etc., the performance of example 1 by diffusion PrDyCu decreased by 0.02 T of Br, increased by 812 kA/m of Hcj compared with the pre-diffusion performance of NdFeB magnet. The performance of comparative example 1 by diffusion Dy decreased by 0.019 T of Br, increased by 653.5 kA/m of Hcj compared with the pre-diffusion performance of NdFeB magnet. Therefore, the Hcj of diffusion PrDyCu increased more significantly and the advantages were more pronounced.
Example 2, with the same NdFeB magnet composition and size, the same diffusion temperature and aging temperature, etc., the performance of example 2 by diffusion PrDyCu decreased by 0.024 T of Br, increased by 699 kA/m of Hcj compared with the pre-diffusion performance of NdFeB magnet. The performance of comparative example 2 by diffusion Dy decreased by 0.023 T of Br, increased by 539.7 kA/m of Hcj compared with the pre-diffusion performance of NdFeB magnet. Therefore, the Hcj of diffusion PrDyCu increased more significantly and the advantages were more pronounced.
Example 3, with the same NdFeB magnet composition and size, the same diffusion temperature and aging temperature, etc., the performance of example 3 by diffusion PrDyCu decreased by 0.022 T of Br, increased by 603.4 kA/m of Hcj compared with the pre-diffusion performance of NdFeB magnet. The performance of comparative example 3 by diffusion Dy decreased by 0.020 T of Br, increased by 404.4 kA/m of Hcj compared with the pre-diffusion performance of NdFeB magnet. Therefore, the Hcj of diffusion PrDyCu increased more significantly and the advantages were more pronounced.
Example 4, with the same NdFeB magnet composition and size, the same diffusion temperature and aging temperature, etc., the performance of example 4 by diffusion PrDyCu decreased by 0.024 T of Br, increased by 598.6 kA/m of Hcj compared with the pre-diffusion performance of NdFeB magnet. The performance of comparative example 4 by diffusion Dy decreased by 0.023 T of Br, increased by 400 kA/m of Hcj compared with the pre-diffusion performance of NdFeB magnet. Therefore, the Hcj of diffusion PrDyCu increased more significantly and the advantages were more pronounced.
Example 5, with the same NdFeB magnet composition and size, the same diffusion temperature and aging temperature, etc., the performance of example 5 by diffusion NdDyCu decreased by 0.025 T of Br, increased by 757 kA/m of Hcj compared with the pre-diffusion performance of NdFeB magnet. The performance of comparative example 5 by diffusion Dy decreased by 0.023 T of Br, increased by 597.8 kA/m of Hcj compared with the pre-diffusion performance of NdFeB magnet. Therefore, the Hcj of diffusion NdDyCu increased more significantly and the advantages were more pronounced.
Example 6, with the same NdFeB magnet composition and size, the same diffusion temperature and aging temperature, etc., the performance of example 6 by diffusion NdDyCu decreased by 0.023 T of Br, increased by 661.5 kA/m of Hcj compared with the pre-diffusion performance of NdFeB magnet. The performance of comparative example 6 by diffusion Dy decreased by 0.021 T of Br, increased by 542 kA/m of Hcj compared with the pre-diffusion performance of NdFeB magnet. Therefore, the Hcj of diffusion NdDyCu increased more significantly and the advantages were more pronounced.
Example 7, with the same NdFeB magnet composition and size, the same diffusion temperature and aging temperature, etc., the performance of example 7 by diffusion NdDyCu decreased by 0.022 T of Br, increased by 702.1 kA/m of Hcj compared with the pre-diffusion performance of NdFeB magnet. The performance of comparative example 7 by diffusion Dy decreased by 0.021 T of Br, increased by 582.7 kA/m of Hcj compared with the pre-diffusion performance of NdFeB magnet. Therefore, the Hcj of diffusion NdDyCu increased more significantly and the advantages were more pronounced.
Example 8, with the same NdFeB magnet composition and size, the same diffusion temperature and aging temperature, etc., the performance of example 8 by diffusion PrDyCu decreased by 0.021 T of Br, increased by 744.3 kA/m of Hcj compared with the pre-diffusion performance of NdFeB magnet. The performance of comparative example 8 by diffusion Dy decreased by 0.019 T of Br, increased by 642.8 kA /m of Hcj compared with the pre-diffusion performance of NdFeB magnet. Therefore, the Hcj of diffusion PrDyCu increased more significantly and the advantages were more pronounced.
Example 9, with the same NdFeB magnet composition and size, the same diffusion temperature and aging temperature, etc., the performance of example 9 by diffusion PrDyCu decreased by 0.024 T of Br, increased by 744.3 kA/m of Hcj compared with the pre-diffusion performance of NdFeB magnet. The performance of comparative example 9 by diffusion Dy decreased by 0.022 T of Br, increased by 585.1 kA/m of Hcj compared with the pre-diffusion performance of NdFeB magnet. Therefore, the Hcj of diffusion PrDyCu increased more significantly and the advantages were more pronounced.
Example 10, with the same NdFeB magnet composition and size, the same diffusion temperature and aging temperature, etc., the performance of example 10 by diffusion PrDyCu decreased by 0.022 T of Br, increased by 786.4 kA/m of Hcj compared with the pre-diffusion performance of NdFeB magnet. The performance of comparative example 10 by diffusion Dy decreased by 0.021T of Br, increased by 627.2 kA/m of Hcj compared with the pre-diffusion performance of NdFeB magnet. Therefore, the Hcj of diffusion PrDyCu increased more significantly and the advantages were more pronounced.
Example 11, with the same NdFeB magnet composition and size, the same diffusion temperature and aging temperature, etc., the performance of example 11 by diffusion PrDyCu decreased by 0.021 T of Br, increased by 616.1 kA/m of Hcj compared with the pre-diffusion performance of NdFeB magnet. The performance of comparative example 11 by diffusion Dy decreased by 0.02 T of Br, increased by 377.3 kA/m of Hcj compared with the pre-diffusion performance of NdFeB magnet. Therefore, the Hcj of diffusion PrDyCu increased more significantly and the advantages were more pronounced.
Example 12, with the same NdFeB magnet composition and size, the same diffusion temperature and aging temperature, etc., the performance of example 12 by diffusion PrDyCu decreased by 0.022 T of Br, increased by 605 kA/m of Hcj compared with the pre-diffusion performance of NdFeB magnet. The performance of comparative example 12 by diffusion Dy decreased by 0.02 T of Br, increased by 406 kA/m of Hcj compared with the pre-diffusion performance of NdFeB magnet. Therefore, the Hcj of diffusion PrDyCu increased more significantly and the advantages were more pronounced.
Example 13, with the same NdFeB magnet composition and size, the same diffusion temperature and aging temperature, etc., the performance of example 13 by diffusion PrDyCuGa decreased by 0.025 T of Br, increased by 605 kA/m of Hcj compared with the pre-diffusion performance of NdFeB magnet. The performance of comparative example 13 by diffusion Dy decreased by 0.023 T of Br, increased by 445.8 kA/m of Hcj compared with the pre-diffusion performance of NdFeB magnet. Therefore, the Hcj of diffusion PrDyCuGa increased more significantly and the advantages were more pronounced.
Example 14, with the same NdFeB magnet composition and size, the same diffusion temperature and aging temperature, etc., the performance of example 14 by diffusion PrDyCuGa decreased by 0.022 T of Br, increased by 656.7 kA/m of Hcj compared with the pre-diffusion performance of NdFeB magnet. The performance of comparative example 14 by diffusion Dy decreased by 0.021 T of Br, increased by 537.3 kA/m of Hcj compared with the pre-diffusion performance of NdFeB magnet. Therefore, the Hcj of diffusion PrDyCuGa increased more significantly and the advantages were more pronounced.
Example 15, with the same NdFeB magnet composition and size, the same diffusion temperature and aging temperature, etc., the performance of example 15 by diffusion PrDyCuGa decreased by 0.025 T of Br, increased by 714.8 kA/m e of Hcj compared with the pre-diffusion performance of NdFeB magnet. The performance of comparative example 15 by diffusion Dy decreased by 0.023 T of Br, increased by 595.4 kA/m of Hcj compared with the pre-diffusion performance of NdFeB magnet. Therefore, the Hcj of diffusion PrDyCuGa increased more significantly and the advantages were more pronounced.
Example 16, with the same NdFeB magnet composition and size, the same diffusion temperature and aging temperature, etc., the performance of example 16 by diffusion PrDyCuAl decreased by 0.023 T of Br, increased by 711.6 kA/m of Hcj compared with the pre-diffusion performance of NdFeB magnet. The performance of comparative example 16 by diffusion Dy decreased by 0.022 T of Br, increased by 592.2 kA/m of Hcj compared with the pre-diffusion performance of NdFeB magnet. Therefore, the Hcj of diffusion PrDyCuAl increased more significantly and the advantages were more pronounced.
Example 17, with the same NdFeB magnet composition and size, the same diffusion temperature and aging temperature, etc., the performance of example 17 by diffusion PrDyCuAl decreased by 0.02 T of Br, increased by 642.4 kA/m of Hcj compared with the pre-diffusion performance of NdFeB magnet. The performance of comparative example 17 by diffusion Dy decreased by 0.02 T of Br, increased by 523 kA/m of Hcj compared with the pre-diffusion performance of NdFeB magnet. Therefore, the Hcj of diffusion PrDyCuAl increased more significantly and the advantages were more pronounced.
Example 18, with the same NdFeB magnet composition and size, the same diffusion temperature and aging temperature, etc., the performance of example 17 by diffusion PrDyCuAl decreased by 0.026 T of Br, increased by 684.6 kA/m of Hcj compared with the pre-diffusion performance of NdFeB magnet. The performance of comparative example 18 by diffusion Dy decreased by 0.025 T of Br, increased by 565.2 kA/m of Hcj compared with the pre-diffusion performance of NdFeB magnet. Therefore, the Hcj of diffusion PrDyCuAl increased more significantly and the advantages were more pronounced.
Example 19, with the same NdFeB magnet composition and size, the same diffusion temperature and aging temperature, etc., the performance of example 19 by diffusion PrDyCu decreased by 0.025 T of Br, increased by 676.6 kA/m of Hcj compared with the pre-diffusion performance of NdFeB magnet. The performance of comparative example 19 by diffusion Dy decreased by 0.024 T of Br, increased by 477.6 kA/m of Hcj compared with the pre-diffusion performance of NdFeB magnet. Therefore, the Hcj of diffusion PrDyCu increased more significantly and the advantages were more pronounced.
Example 20, with the same NdFeB magnet composition and size, the same diffusion temperature and aging temperature, etc., the performance of example 20 by diffusion PrDyCu decreased by 0.02 T of Br, increased by 597kA/m of Hcj compared with the pre-diffusion performance of NdFeB magnet. The performance of comparative example 20 by diffusion Dy decreased by 0.02 T of Br, increased by 477.6 kA/m of Hcj compared with the pre-diffusion performance of NdFeB magnet. Therefore, the Hcj of diffusion PrDyCu increased more significantly and the advantages were more pronounced.
Example 21, with the same NdFeB magnet composition and size, the same diffusion temperature and aging temperature, etc., the performance of example 21 by diffusion PrDyCu decreased by 0.025 T of Br, increased by 756.2 kA/m of Hcj compared with the pre-diffusion performance of NdFeB magnet. The performance of comparative example 21 by diffusion Dy decreased by 0.024 T of Br, increased by 557.2 kA/m of Hcj compared with the pre-diffusion performance of NdFeB magnet. Therefore, the Hcj of diffusion PrDyCu increased more significantly and the advantages were more pronounced.
Example 22, with the same NdFeB magnet composition and size, the same diffusion temperature and aging temperature, etc., the performance of example 22 by diffusion PrDyCu decreased by 0.02 T of Br, increased by 597 kA/m of Hcj compared with the pre-diffusion performance of NdFeB magnet. The performance of comparative example 22 by diffusion Dy decreased by 0.02 T of Br, increased by 398 kA/m of Hcj compared with the pre-diffusion performance of NdFeB magnet. Therefore, the Hcj of diffusion PrDyCu increased more significantly and the advantages were more pronounced.

From the above, it can be seen that after diffusion and aging the coercivity of the examples of Table 3 is significantly better than the coercivity of the comparative examples of Table 4.

Microstructure assays of the magnets of Table 3 are determined by SEM with a ZISS electron microscopy and EDS of Oxford. The following can be seen: A rare earth shell, that is to say, R shell, is around of more than 60% of the grain, and a transition metal shell is around of more than 40% of the grain. In addition, three sampling points (a), (b), (c) are determined at different locations. However, the small triangle area with a size < 1 µm is characterized by a 6:14 phase type rich Cu, that is, the chemical formula of EDS is: Fe₃₀₋₅₁(NdPr)₄₅₋₆₀Cu₂₋₁₅Ga₀₋₅Co₀₋₅ or Fe₃₀₋₅₁(NdPr)₄₅₋₆₀Dy₂₋₁₅Cu₂₋₁₅Ga₀₋₅Co₀₋₅, wherein the number is the percentage of weight at the foot of the element. The three points are shown in Figure 1. White phase area of the point composition a, which is sample point composition 1 are summarized as Formula 1. Grey phase area of the point composition b, which is sample point composition 2 are summarized as Formula 3. Sandwich shape area including heavy rare earth element of the point composition c, which is sample point composition 3 are summarized as Formula 2.
Example 1: The magnet diffused with PrDyCu has the following microstructure: Pr, Dy rare earth shell and transition metal shell Cu, and the formation of sample point composition 1: Nd₅₀₋₇₀Fe₁₀₋₃₀Pr₁₀₋₂₀Cu₀₋₅, sample point composition 2: Nd₅₀₋₇₀Fe₁₀₋₃₅Pr₁₀₋₂₀Cu₁₀₋₂₀Co₀₋₅, sample point composition 3: Nd₅₀₋₅₅Fe₁₀₋₃₀Pr₅₋₁₅Dy₅₋₁₅Cu₀₋₅.
Example 2: The magnet diffused with PrDyCu has the following microstructure: Pr, Dy rare earth shell and transition metal shell Cu, and the formation of sample point composition 1: Nd₅₀₋₆₅Fe₁₀₋₃₀Pr₁₀₋₂₅Cu₀₋₅Ga₀₋₅Al₀₋₃, sample point composition 2: Nd₅₀₋₇₀Fe₁₀₋₃₅Pr₁₀₋₂₀Cu₁₀₋₁₅Co₀₋₅, sample point composition 3: Nd₅₀₋₅₅Fe₁₀₋₃₀Pr₅₋₁₅Dy₅₋₁₅Cu₀₋₅.
Example 3: The magnet diffused with PrDyCu has the following microstructure: Pr, Dy rare earth shell and transition metal shell Cu and Al, and the formation of sample point composition 1: Nd₄₅₋₆₀Fe₁₀₋₃₅Pr₁₀₋₂₀Cu₃₋₈Ga₀₋₅Al₃₋₅, sample point composition 2: Nd₄₅₋₆₅Fe₁₀₋₃₀Pr₁₀₋₂₀Cu₁₀₋₂₅Co₀₋₅Al₀₋₅, sample point composition 3: Nd₄₅₋₅₅Fe₁₀₋₃₀Pr₅₋₂₀Dy₅₋₁₀Cu₂₋₅Al₂₋₁₀
Example 4: The magnet diffused with PrDyCu has the following microstructure: Pr, Dy rare earth shell and transition metal shell Cu and Al, and the formation of sample point composition 1: Nd₄₅₋₆₀Fe₁₀₋₃₅Pr₁₀₋₂₀Cu₃₋₈Ga₀₋₅Al₃₋₅, sample point composition 2: Nd₄₅₋₆₅Fe₁₀₋₃₀Pr₁₀₋₂₀Cu₁₀₋₂₅Co₀₋₅Al₀₋₅, sample point composition 3: Nd₄₅₋₅₅Fe₁₀₋₃₀Pr₅₋₂₀Dy₅₋₁₀Cu₂₋₅Al₂₋₁₀
Example 5: The magnet diffused withNdDyCu has the following microstructure: Nd, Dy rare earth shell and transition metal shell Cu, and the formation of sample point composition 1: Nd₅₀₋₆₅Pr₁₀₋₁₅Fe₁₀₋₃₀Cu₂₋₆Go₀₋₅, sample point composition 2: Nd₄₅₋₆₀Pr₁₀₋₂₀Fe₅₋₃₀Cu₁₀₋₂₀Co₀₋₅, sample point composition 3: Nd₄₅₋₆₀Pr₅₋₁₅Dy₅₋₁₅Fe₅₋₃₀
Example 6: The magnet diffused with NdDyCu has the following microstructure: Nd, Dy rare earth shell and transition metal shell Cu, and the formation of sample point composition 1: Nd₄₅₋₆₀Pr₁₀₋₂₀Fe₁₀₋₃₀Cu₂₋₅Ga₀₋₅ sample point composition 2: Nd₅₀₋₆₀Pr₁₀₋₁₅Fe₅₋₂₅Cu₅₋₂₅Co₀₋₅, sample point composition 3: Nd₄₅₋₆₀Pr₅₋₁₂Dy₅₋₂₀Fe₅₋₂₅
Example 7: The magnet diffused with NdDyCu has the following microstructure: Nd, Dy rare earth shell and transition metal shell Cu and Al, and the formation of sample point composition 1: Nd₅₀₋₆₅Pr₁₀₋₁₅Fe₁₀₋₄₀Cu₅₋₁₀Al₀₋₅ sample point composition 2: Nd₅₀₋₆₀Pr₁₀₋₁₅Fe₅₋₂₅Cu₅₋₁₅Co₀₋₅Al₀₋₅, sample point composition 3: Nd₅₀₋₆₀Pr₅₋₁₅Dy₅₋₂₅Fe₅₋₃₀Al₂₋₁₀
Example 8: The magnet diffused with PrDyCu has the following microstructure: Pr, Dy rare earth shell and transition metal shell Cu, and the formation of sample point composition 1: Nd₄₀₋₆₀Pr₂₀₋₃₀Fe₁₀₋₃₀Cu₃₋₈ sample point composition 2: Nd₃₅₋₅₀Pr₁₅₋₃₀Fe₅₋₂₅Cu₅₋₂₀Co₀₋₅, sample point composition 3: Nd₃₅₋₄₅Pr₁₀₋₂₅Dy₅₋₂₅Fe₁₀₋₃₀Co₀₋₅Cu₀₋₅
Example 9: The magnet diffused with PrDyCu has the following microstructure: Pr, Dy rare earth shell and transition metal shell Cu, and the formation of sample point composition 1: Nd₄₀₋₆₀Pr₂₀₋₃₀Fe₁₀₋₃₀Cu₃₋₈ sample point composition 2: Nd₃₅₋₅₀Pr₁₅₋₃₀Fe₅₋₂₅Cu₅₋₂₀Co₀₋₅, sample point composition 3: Nd₃₅₋₄₅Pr₁₀₋₂₅Dy₅₋₂₅Fe₁₀₋₃₀Co₀₋₅Cu₀₋₅
Example 10: The magnet diffused with PrDyCu has the following microstructure: Pr, Dy rare earth shell and transition metal shell Cu, and the formation of sample point composition 1: Nd₄₀₋₆₀Pr₂₀₋₃₅Fe₁₀₋₃₀Cu₀₋₅ sample point composition 2: Nd₃₅₋₄₅Pr₁₅₋₃₅Fe₅₋₃₀Cu₅₋₂₀Co₀₋₅, sample point composition 3: Nd₂₅₋₄₀Pr₁₀₋₂₅Dy₅₋₁₅Fe₁₀₋₃₀Co₀₋₅Cu₀₋₅
Example 11: The magnet diffused with PrDyCu has the following microstructure: Pr, Dy rare earth shell and transition metal shell Cu, and the formation of sample point composition 1: Nd₅₀₋₆₅Fe₁₀₋₂₅Pr₁₀₋₂₀Cu₀₋₅Ga₀₋₅Al₀₋₅ sample point composition 2: Nd₄₅₋₇₀Fe₁₀₋₃₀Pr₁₀₋₂₅Cu₁₀₋₂₅Co₀₋₅Ga₀₋₅, sample point composition 3: Nd₄₅₋₅₅Fe₁₀₋₃₀Pr₅₋₂₀Dy₅₋₂₀Cu₀₋₅
Example 12: The magnet diffused with PrDyCu has the following microstructure: Pr, Dy rare earth shell and transition metal shell Cu, and the formation of sample point composition 1: Nd₅₀₋₆₅Fe₁₀₋₃₀Pr₁₀₋₂₅Cu₀₋₅Ga₂₋₇Al₃₋₇ sample point composition 2: Nd₅₀₋₆₅Fe₁₀₋₃₅Pr₅₋₂₀Cu₁₀₋₂₀Co₀₋₅Al₀₋₅, sample point composition 3: Nd₄₅₋₅₅Fe₁₀₋₃₀Pr₅₋₂₀Dy₅₋₁₀Cu₀₋₅Ga₀₋₅
Example 13: The magnet diffused with PrDyCuGa has the following microstructure: Pr, Dy rare earth shell and transition metal shell Cu and Ga, and the formation of sample point composition 1: Nd₄₅₋₅₅Pr₂₀₋₂₅Fe₁₅₋₃₀Ga₂₋₁₀Cu₃₋₅ sample point composition 2: Nd₃₅₋₄₅Pr₂₀₋₃₅Fe₁₀₋₃₅Cu₅₋₁₅Ga₅₋₁₀Co₂₋₅, sample point composition 3: Nd₃₀₋₄₅Pr₂₅₋₃₀Dy₅₋₂₀Fe₅₋₂₅Cu₀₋₅
Example 14: The magnet diffused with PrDyCuGa has the following microstructure: Pr, Dy rare earth shell and transition metal shell Cu and Ga, and the formation of sample point composition 1: Nd₄₀₋₅₅Pr₂₀₋₃₀Fe₁₅₋₃₀Ga₂₋₁₀Cu₃₋₅ sample point composition 2: Nd₃₀₋₅₀Pr₂₅₋₃₀Fe₁₀₋₃₀Cu₅₋₁₀Ga₅₋₁₀Co₂₋₅, sample point composition 3: Nd₃₀₋₄₀Pr₂₅₋₃₀Dy₅₋₁₅Fe₅₋₂₅Cu₀₋₅
Example 15: The magnet diffused with PrDyCuGa has the following microstructure: Pr, Dy rare earth shell and transition metal shell Cu and Ga, and the formation of sample point composition 1: Nd₄₀₋₅₅Pr₂₀₋₃₀Fe₁₅₋₂₅Ga₅₋₁₀Cu₃₋₁₀ sample point composition 2: Nd₃₀₋₄₅Pr₂₅₋₃₅Fe₁₀₋₃₀Cu₅₋₁₀Ga₅₋₁₀Co₂₋₅, sample point composition 3: Nd₃₀₋₄₀Pr₁₅₋₃₀Dy₅₋₂₀Fe₅₋₂₅Cu₀₋₅
Example 16: The magnet diffused with PrDyCuAl has the following microstructure: Pr, Dy rare earth shell and transition metal shell Cu and Al, and the formation of sample point composition 1: Nd₄₅₋₆₅Fe₁₀₋₃₅Pr₅₋₁₅Cu₅₋₁₅Al₅₋₁₀ sample point composition 2: Nd₅₀₋₆₅Fe₁₀₋₂₀Pr₁₀₋₁₅Cu₁₀₋₂₅Al₀₋₅, sample point composition 3: Nd₄₅₋₆₅Fe₅₋₃₀Pr₅₋₂₀Dy₅₋₁₀Cu₅₋₁₀Al₂₋₁₀
Example 17: The magnet diffused with PrDyCuAl has the following microstructure: Pr, Dy rare earth shell and transition metal shell Cu and Al, and the formation of sample point composition 1: Nd₄₅₋₅₅Fe₁₀₋₃₀Pr₅₋₂₀Cu₅₋₁₀Al₂₋₅ sample point composition 2: Nd₄₅₋₆₀Fe₁₀₋₂₀Pr₁₀₋₂₀Cu₁₀₋₂₀Ga₀₋₅Al₀₋₅, sample point composition 3: Nd₄₅₋₆₀Fe₅₋₂₅Pr₅₋₂₅Dy₅₋₁₅Cu₅₋₁₀Al₃₋₅
Example 18: The magnet diffused with PrDyCuAl has the following microstructure: Pr, Dy rare earth shell and transition metal shell Cu and Al, and the formation of sample point composition 1: Nd₅₀₋₆₅Fe₁₀₋₃₀Pr₅₋₂₀Cu₅₋₁₀Al₂₋₅ sample point composition 2: Nd₄₅₋₆₀Fe₁₀₋₂₅Pr₁₀₋₂₀Cu₁₀₋₂₀Ga₀₋₅Al₀₋₅, sample point composition 3: Nd₄₅₋₆₅Fe₅₋₃₀Pr₅₋₂₀Dy_{5-15Cu5-10}Al₅₋₁₀
Example 19: The magnet diffused with PrDyCu has the following microstructure: Pr, Dy rare earth shell and transition metal shell Cu, and the formation of sample point composition 1: Nd₄₅₋₅₅Fe₅₋₃₀Pr₂₀₋₃₅Cu₀₋₅ sample point composition 2: Nd₃₅₋₅₅Fe₅₋₃₀Pr₁₀₋₃₅Cu₅₋₁₀Ga₀₋₅Co₀₋₅ sample point composition 3: Nd₄₅₋₅₅Fe₅₋₁₀Pr₁₀₋₃₀Dy₅₋₂₀Cu₀₋₅
Example 20: The magnet diffused with PrDyCu has the following microstructure: Pr, Dy rare earth shell and transition metal shell Cu, and the formation of sample point composition 1: Nd₃₅₋₅₀Fe₁₅₋₄₀Pr₁₅₋₃₀Cu₀₋₁₀Ga₀₋₃Al₀₋₃ sample point composition 2: Nd₄₀₋₅₅Fe₅₋₃₅Pr₁₅₋₃₀Cu₅₋₂₅Ga₀₋₅Co₀₋₅ sample point composition 3: Nd₄₀₋₆₀Fe₃₋₃₀Pr₁₀₋₂₀Dy₅₋₂₅
Example 21: The magnet diffused with PrDyCu has the following microstructure: Pr, Dy rare earth shell and transition metal shell Cu, and the formation of sample point composition 1: Nd₃₀₋₄₅Fe₁₀₋₃₀Pr₂₀₋₂₅Cu₅₋₁₀Ga₀₋₅Co₀₋₅Ti₀₋₅ sample point composition 2: Nd₃₅₋₄₅Fe₅₋₃₀Pr₁₅₋₃₀Cu₅₋₂₅Ga₀₋₃Co₀₋₅ sample point composition 3: Nd₃₀₋₄₀Fe₅₋₂₅Pr₁₀₋₁₅Dy₁₀₋₃₀Ho₅₋₁₀
Example 22: The magnet diffused with PrDyCu has the following microstructure: Pr, Dy rare earth shell and transition metal shell Cu, and the formation of sample point composition 1: Nd₂₅₋₃₅Fe₂₀₋₃₀Pr₂₀₋₃₀Cu₀₋₁₀Ga₀₋₅ sample point composition 2: Nd₄₀₋₅₅Fe₁₀₋₂₅Pr₁₅₋₄₀Cu₅₋₂₀Ga₀₋₁₀Co₀₋₅, sample point composition 3: Nd₄₅₋₅₅Fe₁₀₋₂₀Pr₂₀₋₃₀Dy₅₋₂₀

## Claims

1. A method of preparing a sintered NdFeB magnet comprising the following steps:
(S1) Smelting of the raw materials of a NdFeB alloy to obtain strip casting NdFeB alloy sheets and mechanically crushing the NdFeB alloy sheets into flake alloy sheets, wherein the NdFeB alloy has the following composition in weight percentage:
28%≤R≤30%, 0.8%≤B≤1.2%, 0≤Gd≤5%, 0≤Ho≤5%, and 0≤M≤3%,
where R is at least one element of Nd, Pr, Ce, La, Tb, and Dy,
M is at least one element of Co, Mg, Ti, Zr, Nb, and Mo, and
the rest of the NdFeB alloy is Fe;
(S2) Mechanically mixing the flake alloy sheets, a low melting point powder and a lubricant, followed by hydrogen absorption and dehydrogenation treatment of the mixture and jet milling of the product to obtain a NdFeB magnet powder,
wherein the dehydrogenation temperature is 400 - 600 °C,
wherein the low melting point powder contains at least one component selected form NdCu, NdAl and NdGa and a weight percentage of the components is 0%≤NdCu≤3%, 0%≤NdAl≤3%, and 0%≤NdGa≤3% with respect to the total weight of the flake alloy sheets and the low melting point powder;
(S3) Pressing and forming the NdFeB powder to a blank and sintering the blank to obtain a sintered NdFeB magnet;
(S4) Mechanically processing the sintered NdFeB magnet to a desired shape, and then forming a diffusion source film on the surface of the sintered NdFeB magnet, wherein diffusion source film includes a diffusion source of formula RₓH_{y}M_{1-x-y}, wherein
R is at least one of Nd, Pr, Ce, La, Ho, and Gd,
H is at least one of Tb and Dy,
M is at least one of Al, Cu, Ga, Ti, Co, Mg, Zn, and Sn, and
where x and y are set to be 10%<x≤50% and 40%<y≤70% in weight percentage;
and (S5) Performing a diffusion process and aging to obtain the final sintered NdFeB magnet.

2. The method of claim 1, wherein in step (S2) a weight content of Cu is 0.1%≤Cu≤0.5%, a weight content of Al is 0.2%≤Al≤0.9%, and a weight content of Ga is 0.01%≤Ga≤0.4%, each with respect to the total weight of the flake alloy sheets and the low melting point powder.

3. The method of claim 1 or 2, wherein in the NdFeB alloy of step (S1)
R is at least one element of Nd and Pr, and
M is at least one element of Co and Ti.

4. The method of any one of the preceding claims, wherein in the diffusion source of step (S4)
R is at least one of Nd and Pr,
H is Dy, and
M is at least one of Al, Cu, and Ga.

5. The method of any one of the preceding claims, wherein in step (S2), an average particle size D50 of the low melting point powder is 200 nm - 4 µm measured by laser diffraction (LD).

6. The method of any one of the preceding claims, wherein in step (S2), an average particle size D50 of the NdFeB magnet powder is 3 - 5 µm after jet milling measured by laser diffraction (LD).

7. The method of any one of the preceding claims, wherein in step (S3), the sintering temperature of the NdFeB magnet is 980 - 1060 °C and the sintering time is 6 - 15h.

8. The method of any one of the preceding claims, wherein in step (S5), the diffusion temperature of NdFeB magnets is 850 - 930 °C and the diffusion time is 6 - 30h.

9. The method of any one of the preceding claims, wherein in step (S5), an aging temperature is 420 - 680 °C, an aging time is 3 - 10h, an aging heating rate is 1 - 5 °C/min, and an aging cooling rate is 5 - 20 °C/min.

## Patentansprüche

1. Verfahren zur Herstellung eines gesinterten NdFeB-Magneten, die folgenden Schritte umfassend:
(S1) Schmelzen der Rohmaterialien einer NdFeB-Legierung, um NdFeB-Legierungsbleche im Bandgießverfahren zu erhalten, und mechanisches Zerkleinern der NdFeB-Legierungsbleche in Flockenlegierungsbleche, wobei die NdFeB-Legierung die folgende Zusammensetzung in Gewichtsprozent aufweist:
28 % ≤ R ≤ 30 %, 0,8 % ≤ B ≤ 1,2 %, 0 ≤ Gd ≤ 5 %, 0 ≤ Ho ≤ 5 % und 0 ≤ M ≤ 3 %,
wobei R mindestens ein Element aus Nd, Pr, Ce, La, Tb und Dy ist,
M mindestens ein Element aus Co, Mg, Ti, Zr, Nb und Mo ist, und
der Rest der NdFeB-Legierung Fe ist;
(S2) Mechanisches Mischen der Flockenlegierungsbleche, eines Pulvers mit niedrigem Schmelzpunkt und eines Schmiermittels, gefolgt von einer Wasserstoffabsorptions- und Dehydrierungsbehandlung des Gemischs und Strahlmahlen des Produkts, um ein NdFeB-Magnetpulver zu erhalten, wobei die Dehydrierungstemperatur 400-600 °C beträgt, wobei das Pulver mit niedrigem Schmelzpunkt mindestens eine Komponente enthält, die aus NdCu, NdAl und NdGa ausgewählt ist, und ein Gewichtsprozent der Komponenten 0 % ≤ NdCu ≤ 3 %, 0 % ≤ NdAl ≤ 3 % und 0 % ≤ NdGa ≤ 3 % in Bezug auf das Gesamtgewicht der Flockenlegierungsbleche und des Pulvers mit niedrigem Schmelzpunkt ist;
(S3) Pressen und Ausbilden des NdFeB-Pulvers zu einem Rohling und Sintern des Rohlings, um einen gesinterten NdFeB-Magneten zu erhalten;
(S4) Mechanisches Bearbeiten des gesinterten NdFeB-Magneten zu einer gewünschten Form und anschließendes Bilden eines Diffusionsquellenfilms auf der Oberfläche des gesinterten NdFeB-Magneten, wobei der Diffusionsquellenfilm eine Diffusionsquelle der Formel RₓH_{y}M_{1-x-y} enthält, wobei
R mindestens eines von Nd, Pr, Ce, La, Ho und Gd ist,
H mindestens eines von Tb und Dy ist,
M mindestens eines von Al, Cu, Ga, Ti, Co, Mg, Zn und Sn ist, und
wobei x und y auf 10 %< x ≤ 50 % und 40 % < y ≤ 70 % in Gewichtsprozent festgelegt sind;
und (S5) Durchführen eines Diffusionsprozesses und Alterung, um den endgültigen gesinterten NdFeB-Magneten zu erhalten.

2. Verfahren nach Anspruch 1, wobei in Schritt (S2) ein Gewichtsanteil von Cu 0,1 % ≤ Cu ≤ 0,5 %, ein Gewichtsanteil von Al 0,2 % ≤ Al ≤ 0,9 % und ein Gewichtsanteil von Ga 0,01 % ≤ Ga ≤ 0,4 % beträgt, jeweils bezogen auf das Gesamtgewicht der Flockenlegierungsbleche und des Pulvers mit niedrigem Schmelzpunkt.

3. Verfahren nach Anspruch 1 oder 2, wobei in der NdFeB-Legierung von Schritt (S1)
R mindestens ein Element aus Nd und Pr ist, und
M mindestens ein Element aus Co und Ti ist.

4. Verfahren nach einem der vorhergehenden Ansprüche, wobei in der Diffusionsquelle von Schritt (S4)
R mindestens eines von Nd und Pr ist,
H Dy ist, und
M mindestens eines von Al, Cu und Ga ist.

5. Verfahren nach einem der vorhergehenden Ansprüche, wobei in Schritt (S2) eine durchschnittliche Partikelgröße D50 des Pulvers mit niedrigem Schmelzpunkt 200 nm - 4 µm beträgt, gemessen durch Laserbeugung (LD).

6. Verfahren nach einem der vorhergehenden Ansprüche, wobei in Schritt (S2) eine durchschnittliche Partikelgröße D50 des NdFeB-Magnetpulvers nach dem Strahlmahlen 3-5 µm beträgt, gemessen durch Laserbeugung (LD).

7. Verfahren nach einem der vorhergehenden Ansprüche, wobei in Schritt (S3) die Sintertemperatur des NdFeB-Magneten 980-1060 °C und die Sinterzeit 6-15 h beträgt.

8. Verfahren nach einem der vorhergehenden Ansprüche, wobei in Schritt (S5) die Diffusionstemperatur der NdFeB-Magnete 850-930 °C und die Diffusionszeit 6-30 h beträgt.

9. Verfahren nach einem der vorhergehenden Ansprüche, wobei in Schritt (S5) eine Alterungstemperatur 420-680 °C, eine Alterungszeit 3-10 h, eine Alterungsheizrate 1-5 °C/min und eine Alterungskühlrate 5-20 °C/min betragen.

## Revendications

1. Procédé de préparation d'un aimant de NdFeB fritté comprenant les étapes suivantes :
(S1) Fusionner des matières premières d'un alliage de NdFeB pour obtenir des feuilles d'alliage de NdFeB coulées en bandes et broyer mécaniquement des feuilles d'alliage de NdFeB en feuilles d'alliage de flocons, l'alliage de NdFeB ayant la composition suivante en pourcentage en poids :
28 % ≤ R ≤ 30 %, 0,8 % ≤ B ≤ 1,2 %, 0 ≤ Gd ≤ 5 %, 0 ≤ Ho ≤ 5 %, et 0 ≤ M ≤ 3 %,
dans lequel R est au moins un élément de Nd, Pr, Ce, La, Tb et Dy,
dans lequel M est au moins un élément de Co, Mg, Ti, Zr, Nb et Mo, et
dans lequel le reste de l'alliage de NdFeB est constitué de Fe ;
(S2) Mélanger mécaniquement des feuilles d'alliage de flocons, d'une poudre à bas point de fusion et d'un lubrifiant, suivi d'un traitement d'absorption d'hydrogène et de déshydrogénation du mélange et d'un broyage à jet du produit pour obtenir une poudre d'aimant de NdFeB, la température de déshydrogénation étant comprise entre 400 et 600 °C, la poudre à bas point de fusion contenant au moins un composant choisi parmi NdCu, NdAl et NdGa et un pourcentage en poids des composants étant de 0 % ≤ NdCu ≤ 3 %, 0 % ≤ NdAl ≤ 3 % et 0 % ≤ NdGa ≤ 3 % par rapport au poids total des feuilles d'alliage de flocons et de la poudre à bas point de fusion ;
(S3) Presser et former la poudre de NdFeB en une ébauche et fritter l'ébauche pour obtenir un aimant de NdFeB fritté ;
(S4) Traiter mécaniquement l'aimant de NdFeB fritté jusqu'à une forme souhaitée, puis former un film de source de diffusion sur la surface de l'aimant de NdFeB fritté, le film de source de diffusion comprenant une source de diffusion de formule RₓH_{y}M_{1-x-y}, dans lequel
R est au moins un élément de Nd, Pr, Ce, La, Ho et Gd,
H est au moins un élément de Tb et Dy,
M est au moins un élément d'Al, Cu, Ga, Ti, Co, Mg, Zn et Sn, et
dans lequel x et y sont fixés à 10 % < x ≤ 50 % et 40 % < y ≤ 70 % en pourcentage en poids ;
et (S5) Réaliser un processus de diffusion et de vieillissement pour obtenir l'aimant de NdFeB fritté final.

2. Procédé de la revendication 1, dans lequel à l'étape (S2) une teneur en poids de Cu est de 0,1 % ≤ Cu ≤ 0,5 %, une teneur en poids d'Al est de 0,2 % ≤ Al ≤ 0,9 %, et une teneur en poids de Ga est de 0,01 % ≤ Ga ≤ 0,4 %, chacune par rapport au poids total des feuilles d'alliage de flocons et de la poudre à bas point de fusion.

3. Procédé de la revendication 1 ou 2, dans lequel dans l'alliage de NdFeB de l'étape (S1)
R est au moins un élément de Nd et Pr, et
M est au moins un élément de Co et Ti.

4. Procédé de l'une quelconque des revendications précédentes, dans lequel dans la source de diffusion de l'étape (S4).
R est au moins un élément de Nd et Pr,
H est Dy, et
M est au moins un élément d'Al, Cu et Ga.

5. Procédé de l'une quelconque des revendications précédentes, dans lequel à l'étape (S2), une taille moyenne de particule D50 de la poudre à bas point de fusion est comprise entre 200 nm - 4 µm mesurée par diffraction laser (LD).

6. Procédé de l'une quelconque des revendications précédentes, dans lequel à l'étape (S2), une taille moyenne de particule D50 de la poudre d'aimant de NdFeB est comprise entre 3 à 5 µm après le broyage à jet, mesurée par diffraction laser (LD).

7. Procédé de l'une quelconque des revendications précédentes, dans lequel, à l'étape (S3), la température de frittage de l'aimant de NdFeB est comprise entre 980 - 1060 °C et la durée de frittage est comprise entre 6 - 15 h.

8. Procédé de l'une quelconque des revendications précédentes, dans lequel à l'étape (S5), la température de diffusion des aimants de NdFeB est comprise entre 850 et 930 °C et la durée de diffusion est comprise entre 6 et 30 h.

9. Procédé de l'une quelconque des revendications précédentes, dans lequel, à l'étape (S5), la température de vieillissement est comprise entre 420 et 680 °C, la durée de vieillissement est comprise entre 3 et 10 h, la vitesse de chauffage de vieillissement est comprise entre 1 et 5 °C/min et la vitesse de refroidissement de vieillissement est comprise entre 5 et 20 °C/min.
